

## UNITED STATES PATENT OFFICE

2,242,239

## METHOD OF CENTRIFUGAL CASTING

Walter G. Donald, Cambridge, and James L. Martin, Lowell, Mass.

No Drawing. Application December 19, 1938,  
Serial No. 246,646

5 Claims. (Cl. 22—65)

(Granted under the act of March 3, 1883, as  
amended April 30, 1928; 370 O. G. 757)

The invention described herein may be manufactured and used by or for the Government for governmental purposes, without the payment to us of any royalty thereon.

This invention relates to a method of centrifugally casting iron in chill molds and more particularly to controlling the gradient from white iron to gray iron in cylindrical or similar cast iron castings of the class having an outside diameter on the order of four to six times the inside diameter or equivalent wall thickness which class will hereinafter be referred to generally as thick-walled cylinders or castings.

Heretofore, where the need has arisen for thick walled cylinders or castings capable of at once withstanding high pressures and offering a wear and corrosion resistant interior surface, it has been necessary to either compromise on a single material not complying with the full requirements of the need, or to use concentrically bonded materials wherein trouble has been experienced in obtaining a satisfactory bond.

This necessity has existed because of the difficulty in avoiding segregation during freezing of the large volume of metal used in thick-walled cylinders, or similar castings which causes the actual composition of the metal to widely vary in different portions of the casting. If the molten metal or heat is poured into an ordinary stationary chill mold of a size to give a thick-walled casting of any appreciable length, both longitudinal and transverse segregation results which is either exceedingly difficult or impossible to control within economically feasible limits, this being especially true of longitudinal segregation. On the other hand longitudinal segregation is avoided in the usual centrifugal cast iron castings as made in the art at present, but such castings are so relatively thin-walled that little if any gradient of composition of any type results in the casting, consequently the fabrication of a thick-walled cylindrical or similar member of two or more such castings concentrically or contiguously arranged does not result in a structure having a uniform gradient from the outer surface of the casting to the bore or inner side thereof.

It is an object of this invention to set forth a method for casting thick-walled cast iron cylindrical or similar castings which incorporates steps heretofore employed for chilling the surfaces of similar castings of short length; such as railway car wheels and mill rolls, with present known centrifugal casting methods, in order to eliminate longitudinal segregation, and thereby

render available an economical method of producing castings of this class in substantial lengths.

It is a further object of this invention to control the radial segregation of carbon in thick-walled centrifugal castings by controlling the amount of carbon in the composition of metal being cast to effect a predetermined gradient from white iron to gray iron.

10 While the essential objects and steps of this invention have been outlined above the same consists particularly in the steps to be hereinafter set forth, it being understood however, that the description is for the purpose of illustration and 15 no limitation.

If a thick-walled cast iron cylinder or similar casting be cast centrifugally in a horizontally disposed cylindrical or other appropriate chill mold spun about its longitudinal axis under conditions insuring a continuous uniform flow of molten metal throughout the full length of the mold, longitudinal segregation will be eliminated due to the radial action of centrifugal force upon the flowing metal. At the same time, however, 20 due to the solidification process and/or centrifugal force radial segregation of the carbon and other elements or impurities will be effected, and it is the control of this radial segregation of carbon, through a control of the total carbon content of the composition being cast that we have provided for regulating the gradient from white iron to gray iron in thick-walled cylindrical or 25 similar castings.

We have found that since segregation is not 30 due to centrifugal force alone; but, is also effected by the solidification process through which the molten metal passes in freezing, that there are several factors in any given set of conditions 35 affecting the solidification process that must be maintained constant in order to obtain a desired gradient from white iron to gray iron solely through control of the total carbon in the composition. These factors are:

1. The chill ratio between the mold and casting 40 must be kept constant; i. e., the ratio between the cross-sectional area of the mold and cross-sectional area of the casting must be maintained constant,

2. The pouring temperature of the pour must 45 be kept constant, and finally,

3. The composition of the pour aside from the 50 carbon content must be kept constant.

By maintaining the three above enumerated factors constant we have found that castings varying from all white iron with 2.5% carbon to

practically all gray iron with approximately 4.0% carbon may be cast in accordance with a predetermined specification through control of the carbon content of the molten metal to be cast. By increasing the carbon in steps above 2.5%, the outer white iron ring or zone becomes less in depth and the inner gray iron ring or zone becomes correspondingly greater in depth, owing to the fact that the carbon is physically displaced inwardly by the process of solidification and centrifugal force.

The method of this invention avoids or eliminates the longitudinal or top segregation characteristic of castings made in stationary chill molds, provides castings having the desirable density characteristic of centrifugal castings, and teaches a method of coordinating the radial segregating action of centrifugal force and the solidification process for a more accurate control of the radial carbon gradient than has hitherto been possible.

As examples of the control that may be attained of the depth of the white iron ring or zone, through variation in the total carbon content of the melt alone, when the remaining factors above enumerated are kept constant the following is given for a composition which except for carbon is otherwise constant.

| Ex. No. | Radial thickness of section in inches | C. percent | Pour temp. in degrees Fahrenheit | Chill ratio | Depth of white iron zone or ring in inches | Depth of gray iron ring or zone in inches |
|---------|---------------------------------------|------------|----------------------------------|-------------|--------------------------------------------|-------------------------------------------|
| 1.....  | 2.0                                   | 2.70       | 2950                             | 6.5         | 2.00                                       | -----                                     |
| 2.....  | 2.0                                   | 3.10       | 2950                             | 6.5         | 1.70                                       | 0.30                                      |
| 3.....  | 2.0                                   | 3.65       | 2950                             | 6.5         | 1.55                                       | 0.45                                      |

It will be noted that the depth of the white iron ring or zone is changed through a control of total carbon alone and that it is not necessary to otherwise relatively change the proportions of the silicon and sulphur with respect to the carbon to regulate this ring or zone.

Having thus described our invention, what we claim and desire to secure by Letters Patent is:

We claim:

1. In the method of centrifugally chill casting thick-walled cast iron castings of the class having an outside diameter of four to six times the inside diameter and of appreciable length and uniform composition except as to carbon and predetermined the depth of white iron zone formed therein through regulation of the carbon content of the iron to be cast, the steps which comprise employing a horizontally disposed chill mold rotating on its longitudinal axis and having a cross-sectional area with respect to the cross-sectional area of the casting proportioned in the ratio of 6.5:1 to dissipate heat therefrom at a rate effective to control radial segregation of carbon in a casting of the class recited varying from all white iron with 2.5% carbon to substantially all gray iron with 4.0% carbon, introducing in said mold an iron at constant temperature with a carbon content between the limits of 2.5% and 4.0% in accordance with the depth of white iron zone determined to eliminate longitudinal segregation, and maintaining rotation of the mold from the time of introduction of the iron until solidification.

2. In the method of centrifugally chill casting thick-walled cast iron castings of the class having an outside diameter of 4 to 6 times the inside diameter and of uniform composition except as to carbon and predetermined the depth of white iron zone formed therein through regulation of the carbon content of the iron to be cast alone, the steps which comprise selecting a rotating chill mold having its cross-sectional area proportioned with respect to the cross-sectional area of the casting in a chill ratio adapted to dissipate heat therefrom at a rate effective to control radial segregation of carbon in a casting of the class recited varying from all white iron with 2.5% carbon to substantially all gray iron with 4.0% carbon, correlating the carbon content of an iron with the depth of white iron zone predetermined for the casting and the chill ratio between the limits of 2.5% and 4.0%, introducing said iron in the mold, and maintaining rotation of the mold until solidification of the casting.

3. In the method of forming cast iron cylindrical tubular articles of the class having an outside diameter of 4 to 6 times the inside diameter, the steps which comprise providing a rotatable chill mold having its cross-sectional area proportioned with respect to the cross-sectional area of a tubular article of said diameters in a ratio between the limits of 6.5:1 and 1:1, selecting a cast iron, solely regulating the carbon content of said iron to a point between the limits of 2.5% to 4.0% in accordance with said ratio and a predetermined depth of white iron zone to be formed in the article between the limits of 0% and 100%, rotating the mold, and pouring said iron in molten form into the mold at a constant temperature.

4. In the method of forming cast iron cylindrical tubular articles of the class having an outside diameter of 4 to 6 times the inside diameter, the steps which comprise providing a rotatable chill mold having its cross-sectional area proportioned with respect to the cross-sectional area of a tubular article of said diameters in a ratio of 6.5:1, selecting a cast iron, solely regulating the carbon content of said iron to a point between the limits of 2.5% to 4.0% in accordance with said ratio and a predetermined depth of white iron zone to be formed in the article between the limits of 0% and 100%, rotating the mold, and pouring said iron in molten form into the mold at a constant temperature.

5. In the method of forming cast iron cylindrical tubular articles of the class having a radial thickness of 2 inches, the steps which comprise providing a rotatable chill mold having its cross-sectional area proportioned with respect to the cross-sectional area of a tubular article of radial thickness of two inches in the ratio of 6.5:1, selecting a cast iron, solely regulating the carbon content of the iron to a point between the limits of 2.70% to 3.65% in correlation with a predetermined depth of white iron zone to be formed in the article between the limits of 2.0 inches and 1.55 inches and said ratio of 6.5:1, rotating the mold, and pouring said iron in molten form into the mold at a temperature of 2950° F.

WALTER G. DONALD.  
JAMES L. MARTIN.